

## UNITED STATES PATENT OFFICE

1,921,920

PROCESS FOR OBTAINING RESERVES  
UNDER AZO-DYESTUFFSRobert Haller, Riehen, near Basel, Switzerland,  
assignor to Society of Chemical Industry in  
Basle, Basel, SwitzerlandNo Drawing. Application July 7, 1932, Serial  
No. 621,310, and in Switzerland July 23, 1931

8 Claims. (Cl. 8-5)

The present invention relates to the production of white and colored reserves under such azo-dyestuffs which are obtained by treating fibers impregnated with coupling components, with diazo-5 compounds.

It has been found that the property of the xanthogenates to react very easily with diazo-compounds is excellently adapted to prevent the formation of azo-dyestuffs capable of being obtained from the components on the fiber. The process is carried out by printing thickened solutions of salts of xanthogenic acid on textiles, preferably after they have in normal manner been prepared with coupling components, and then 10 producing the azo-dyestuff by treatment with a solution of a suitable diazotized amine. In this manner clear white reserves are obtained. The treatment may also be performed in such a manner that the salts of the xanthogenic acid are 15 printed on the untreated goods, then treating the goods with a coupling component, and, after drying, effecting the development in a bath of the diazo solution.

As coupling components there come quite generally into consideration all products which have been recommended for the production of insoluble azo-dyestuffs, for example  $\beta$ -naphthol, the arylides of  $\beta$ -hydroxynaphthoic acid and the derivatives thereof capable of being coupled in 1-position, the arylides of other acids, such as those of the hydroxycarbazol, hydroxyphenanthrene, hydroxydiphenylamine, and hydroxyanthracene carboxylic acids, coupling components with the  $\text{CH}_2\text{CO}$  group, such as pyrazolone, acetoacetic derivatives, such as, for example, the arylides 30 from acetoacetic acid, bases of the diphenyl series, such as benzidine, tolidine and dianisidine, further 1-hydroxynaphthalene-4-arylketones, arylides of phenol carboxylic acids, such as arylides of the p-kresotinic acid or of xylanol carboxylic acids capable of being coupled, etc.

As suitable diazotizable amines there may be mentioned the unsulfonated aromatic diazo-compounds which have also been recommended for 45 the production of insoluble dyestuffs on the fiber, for example aniline, chloro- and nitroanilines, chloro-, nitro- and chloronitrotoluidines, monoacylated p-, o-, and m-phenylenediamines, aminodiarylethers, aminodiphenylamines,  $\alpha$ - and  $\beta$ -naphthylamines, aminoanthraquinones, amino-50 carbazoles, aminoazo-compounds, etc.

It has further been found that in an analogous manner colored reserves may be produced under azo-dyestuffs by incorporating dyestuffs into the 55 reserve containing xanthogenate, which dyestuffs

are then fixed on the fabric without influencing the reserving effect of the xanthogenate in any way.

As salts of the xanthogenic acid there are preferably used the alkali metal salts, but also other salts, for example heavy metal salts, such as tin or zinc, or other metal salts, such as magnesium or aluminium salts. Such salts are preferably formed in the printing color by conversion of the alkali xanthogenates with salts of other metals. 60

For producing colored reservations, dyestuffs (this term including leuco compounds of vat dyestuffs) which are capable of fixing on the goods are added to the printing paste containing the salt of the xanthogenic acid, and printed. 65

For producing colored reservations basic dyestuffs and vat dyestuffs are particularly suitable, the latter may also be applied in the form of their leuco compounds, this expression including the leuco derivatives, the leuco ester salts, the leuco ethers (cf. British Patent No. 291,763) etc., respectively. The leuco compounds, after combination of the coupling component with the diazotized amine, are then transformed in the usual manner into the corresponding dyestuffs. 70

The following examples illustrate some methods of realization of the present invention, it being obvious that numerous other possibilities are possible still, the feature of the invention being, as already mentioned, the local destruction of the diazo compound on the fiber, due to the presence of the salts of the xanthogenic acid, it being inter alia irrelevant in which manner the colored effects, if any, are produced at the reserved places:— 80

## Example 1

The fabric is impregnated with a solution of 12 g. of 2:3-hydroxynaphthoic acid anilide 10 ccm. of caustic soda solution of 36° Bé. 95 15 ccm. of Turkey red oil of 50 per cent. strength 300 ccm. of hot water, adjusted to

1000 ccm. and the dried material is printed with the following printing color: 100

125 g. of a solution of gum 1:1 50 g. of potassium xanthogenate 50 ccm. of water 105

The goods are then dried again, and developed in the solution of a diazo-salt from 4-chlor-2-aminodiphenyl ether. White effects on a red ground are thus obtained. 110

*Example 2*

The material impregnated according to Example 1 is printed with the following colored reserve:—

5 12 g. of Indigosol 04B (Schultz, Leipzig 1931, No. 1314)

50 ccm. of water (heated until dissolved and then cooled)

125 g. of gum 1:1

10 50 g. of potassium xanthogenate

The goods are then developed in a diazo solution containing per liter 12 g. of diazotized 4-nitro-3:6-dimethyl-1-aminobenzene, and immediately afterwards passed through a bath of

15 5 g. of sodium nitrite

20 20 ccm. of hydrochloric acid of 22° Bé., adjusted to

20 1000 ccm. of water

Blue effects on a red ground are thus obtained.

*Example 3*

The fabric is prepared with

25 15 g. of benzoyl-1-hydroxynaphthalene

15 ccm. of caustic soda solution of 36° Bé.

15 ccm. of Turkey red oil of 50 per cent. strength

300 ccm. of boiling water, adjusted to

30 1000 ccm.

and then printed with a printing color prepared as follows:—

135 g. of gum 1:1

35 12.5 g. of Ciba blue 2BD paste (Schultz, Leipzig 1931, No. 1314)

12.5 g. of potash, and

10 g. of concentrated hydrosulfite powder are heated together until reduction has taken place, cooled down and

40 50 g. of potassium xanthogenate added

The material is then steamed for 3 to 4 minutes in the quick steamer and developed in a solution containing per liter 60 g. of a diazo-salt from 4-chloro-2-aminodiphenyl ether, (corresponding to 12 grams of 4-chloro-2-aminodiphenyl ether per liter). Blue effects on a red ground are thus obtained.

*Example 4*

The fabric is impregnated with a solution of

50 12 g. of 2:3-hydroxynaphthoic acid anilide

18 ccm. of caustic soda solution of 36° Bé.

15 ccm. of Turkey red oil of 50 per cent strength

55 300 ccm. of hot water

12 g. of Katanol O, (cf. Dr. P. Heermann, Technologie der Textilveredlung, Berlin 1926, page 164) adjusted to

60 1000 ccm.

and the dried fabric is printed with

65 2.5 g. of Methylene blue D (Schultz, Leipzig 1931, No. 1038)

5 ccm. of alcohol

45 ccm. of water

125 g. of gum 1:1

50 g. of potassium xanthogenate.

70 The material is then developed in a solution containing per liter 50 g. of a diazo-salt from 4-chloro-2-aminodiphenyl ether (corresponding to 10 grams of 4-chloro-2-aminodiphenyl ether per liter), followed by washing and soaping. Blue

75 effects on a red ground are thus obtained.

*Example 5*

The fabric is impregnated with the following solution:

25 g. of di-acetoacetic toolidide

20 ccm. of caustic soda solution of 38° Bé. 80

20 ccm. of Turkey red oil of 50 per cent strength, adjusted to

1000 ccm. 85

The material is then printed with the resist prepared as per Example 1, and developed in a bath containing per liter 75 g. of a diazo preparation from m-nitro-p-toluidine (corresponding to 15 g. of meta-nitro-p-toluidine per liter). White effects on a yellow ground are thus obtained. 90

*Example 6*

The fabric is impregnated as indicated in Example 1 with 12 g. of 2:3-hydroxynaphthoic acid anilide, and then printed with the following resist: 95

125 g. of gum 1:1

50 g. of potassium xanthogenate

40 g. of stannous chloride

50 ccm. of water. 100

After drying, the material is developed in a bath containing 24 g. of a diazo-preparation from 4-amino-4'-ethoxydiphenyl amine of 40 per cent. strength. White effects on a blue ground are thus obtained. 105

*Example 7*

The fabric is impregnated with 15 g. of the product known in the trade by the name Naphthol ASLB (cf. Textile Colorist, 1931, page 561), printed with the resist prepared according to Example 6, and developed in a diazo-bath containing per liter 12 g. of the diazo-compound of 5-nitro-o-anisidine. White effects on a brown ground are thus obtained. 115

What I claim is:—

1. Process for the production of reserves under azo-dyestuffs which are obtained by treating with diazo-compounds goods prepared with coupling components, consisting in printing the goods with a metal salt of xanthogenic acid prior to the treatment with the diazo-compound. 120

2. Process for the production of reserves under azo-dyestuffs which are obtained by treating with diazo-compounds goods prepared with coupling components, consisting in printing the goods with an alkali metal salt of xanthogenic acid prior to the treatment with the diazo-compound. 125

3. Process for the production of reserves under azo-dyestuffs which are obtained by treating with diazo-compounds goods prepared with coupling components, consisting in printing the goods prepared with the coupling component with a metal salt of xanthogenic acid prior to the treatment with the diazo-compound. 130

4. Process for the production of reserves under azo-dyestuffs which are obtained by treating with diazo-compounds goods prepared with coupling components, consisting in printing the goods prepared with the coupling component with an alkali metal salt of xanthogenic acid prior to the treatment with the diazo-compound. 135

5. Process for the production of reserves under azo-dyestuffs which are obtained by treating with diazo-compounds goods prepared with coupling components, consisting in printing the goods with a salt of xanthogenic acid together with a dye-stuff which is capable of fixing on the goods, prior to the treatment with the diazo-compounds. 145

6. Process for the production of reserves under 150

azo-dyestuffs which are obtained by treating with diazo-compounds goods prepared with coupling components, consisting in printing the goods with an alkali metal salt of xanthogenic acid together with a dyestuff which is capable of fixing on the goods, prior to the treatment with the diazo-compound.

5

7. Process for the production of reserves under azo-dyestuffs which are obtained by treating with diazo-compounds goods prepared with coupling components, consisting in printing the goods with a salt of xanthogenic acid together with a leuco-

compound of a vat dyestuff which is capable of fixing on the goods, prior to the treatment with the diazo-compound.

8. Process for the production of reserves under azo-dyestuffs which are obtained by treating with diazo-compounds goods prepared with coupling components, consisting in printing the goods with an alkali metal salt of xanthogenic acid together with a leuco-compound of a vat dyestuff which is capable of fixing on the goods, prior to the treatment with the diazo-compounds.

ROBERT HALLER.

|    |     |
|----|-----|
| 15 | 90  |
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |